# EUROPEAN PATENT SPECIFICATION

(11) **EP 2 776 782 B1**
(45) Date of publication and mention of the grant of the patent: **06.04.2016**
(21) Application number: 12798897.0
(22) Date of filing: 25.10.2012
(51) Int. Cl.: F41H 5/04

(54) **COMPOSITE PASSIVE ARMOR PROTECTION**
PASSIVER VERBUNDSCHUTZPANZER
PROTECTION À BLINDAGE PASSIF COMPOSITE

(30) Priority: 07.11.2011 PL 39689611
(43) Date of publication of application: 17.09.2014
(73) Proprietor: Instytut Odlewnictwa, 30-418 Kraków (PL)
(72) Inventor: SOBCZAK, Jerzy, PL-32-020 Wieliczka (PL); DARlAK, Pawel, PL-30-820 Kraków (PL); DLUGOSZ, Piotr, PL-31-636 Kraków (PL)
(74) Representative: Bartula-Toch, Marta
(86) International application number: PCT/PL2012/000117
(87) International publication number: WO 2013/070100

(56) References cited:
- DE-A1- 1 578 324
- US-A1- 2007 017 359
- US-B1- 7 833 627

## Description

The invention relates to a composite passive armor protection to safeguard objects from the effect of projectiles and projectile fragments.

As known from the DE1578324 description of armor, the energy-absorbing elements are embedded in a non-metallic matrix. Elements, having the shape of cylindrical bodies, are arranged in layers and placed next to each other or at certain distances. On the other hand, the protective screen to defend against explosion as disclosed in the PL171251 description is made of air-permeable side layers, having the form of precut sheets of metal foil, and of a porous core, placed between these foils, containing the beads or ellipsoids made of the same material as the sheet. Preferably, the sheets of metal foil contain magnesium alloy. A passive armor known from the PL181177 description consists of the main inner protective metal layer and the outer protective layer comprising a number of rectangular, metallic cassettes containing ceramic layers. The spaces between the ceramic layers and the surfaces of the cassette walls are filled with a composition of small ceramic pieces mixed with glue and concrete. The cassettes in an outer protective layer of the armor are removably secured to the main inner protective metal layer by means of various connecting and clamping elements. A safety element used to protect the life and health of the crew of a military vehicle against the explosion of mine under this vehicle known from the PL206571 description consists of a shield having through-holes on its entire surface. The shield is connected by means of the vertical supports with a thin intermediate plate, which, through springs and connected to these springs mounting plates, is attached to the underside of the vehicle floor. Discharge ducts are running from the shield surface. Patent specification US 7, 833, 627 , which forms the starting point for claim 1, discloses a composite armor having a layered metallic matrix structure with embedded ceramic elements, whereby the embedment ceramic elements are situated at an interface between the first inner casting and the second outer casting.

The composite passive armor protection according to the present invention comprises the features of claim 1.

The grooves in the upper plate are made in such a way that their axes coincide with the axes of the geometric solids resting in these grooves. Adventaugosly, the geometric solids are spheres or truncated pyramids with a square base.

The geometric solids are ceramic or metallic solids.

Owing to its specific construction, the composite passive armor protection according to the present invention is resistant to projectile impacts. The protruding part of geometric solids prevents the penetration of AP-type projectiles, projectile fragments, and small arms projectiles. The mere shape and very hard material of the geometric solids cause distortion in the projectile flight path, or ricochet and weakening of the projectile kinetic energy. The layer between the plates, filled with the light alloy matrix material, forms an energy gap limiting crack propagation and resulting in dissipation of the kinetic energy of the projectile. The task of the bottom plate is to completely arrest the projectile, the energy of which was reduced on the layer of the geometric solids resting on the grooved upper plate and in the energy gap. Additionally, the grooves in the upper plate prevent movement of the geometric solids in respect of the plate surface. The light alloy matrix protects the armor against tearing. The composite passive armor protection according to the present invention, the matrix whereof is made of a light alloy, is highly effective in protection against the AP projectiles of up to 12.6 mm. The use of light alloy as a matrix material reduces the armor weight, thereby increasing the mobility of the protected vehicles, reducing fuel consumption and enabling the armor to be used as a means of protection for the aircraft and watercraft.

The composite passive armor protection according to the present invention is shown in a sample embodiment in the accompanying drawings, where Figure 1 shows a vertical section of the composite passive armor protection, and Figure 2 its schematic representation.

The composite passive armor protection consists of two parallel plates 1 and 2, except that in the grooves 3 in the upper plate 1 are resting balls 4 embedded in the light alloy matrix 5 up to a level of the two-third of their diameter. Between the plates 1 and 2 there is a separating layer 6 made of a light alloy 5, wherein said layer is forming an energy gap.

## Claims

1. A composite passive armor protection having geometric solids embedded in a matrix, wherein the armor protection comprises parallel non-adjacent plates (1) and (2), wherein the upper plate (1) has grooves (3), in which are resting the geometric solids (4) embedded in a light alloy matrix (5) to a level above one half of their total height leaving a part of the geometric solids (4) protruding, while the space between the parallel plates is a layer of light alloy (6).

2. The composite passive armor protection of claim 1, wherein the axes of the grooves (3) in the upper plate (1) coincide with the axes of the geometric solids (4) resting in these grooves (3).

3. The composite passive armor protection of claim 1, wherein said geometric solids (4) are ceramic solids or metallic solids.

4. The composite passive armor protection of claim 1, wherein said geometric solids (4) are in the shape of spheres or truncated pyramids with a square base.

## Patentansprüche

1. Passiver Verbundgussschutzpanzer, der in der Matrix eingeschmolzene geometrischen Körper besitzt ist **dadurch gekennzeichnet, dass** er aus parallelen nicht anliegenden Platten 1 und 2 gebaut ist, wo obere Platte 1 Aussparungen 3 hat in deren sich, günstig bis an Niveau über die Hälfte der ganzen ihren Höhe, eingeschmolzene in der Matrix aus Leichtmetalllegierung 5 geometrischen Körper 4 befinden und zwar so, dass ein Teil von geometrischen Körpern 4 herausragt und den Abstand zwischen den parallelen Platen bildet die Schicht aus der Leichtmetalllegierung 6.

2. Passiver Verbundgussschutzpanzer nach Anspruch 1 ist **dadurch gekennzeichnet, dass** die Achsen der Aussparungen 3 in der oberen Platte 1 mit den Achsen sich in den Aussparungen 3 befindenden Körpern 4 übereinstimmen.

3. Passiver Verbundgussschutzpanzer nach Anspruch 1 ist **dadurch gekennzeichnet, dass** die geometrischen Körper 4 aus Keramik oder Metall sind.

4. Passiver Verbundgussschutzpanzer nach Anspruch 1 ist **dadurch gekennzeichnet, dass** die geometrischen Körper 4 eine Kugel- oder Pyramidenstumpfgestalt mit einer quadranttischen Grundfläche haben.

## Revendications

1. Blindage de protection passif en composite, muni de solides géométriques noyés dans une matrice, **caractérisé en ce qu'**il est constitué de plaques parallèles non contigues 1 et 2, étant précisé que la plaque supérieure 1 possède des rainures 3, dans lesquelles sont installés les solides géométriques 4 noyés dans la matrice en alliage léger 5, de préférence jusqu'au-dessus de la moitié de leur hauteur totale, de sorte qu'une partie des solides géométriques 4 fait saillie et l'espace entre les plaques parallèles forme une couche en alliage léger 6.

2. Blindage de protection passif en composite selon la revendication 1, **caractérisé en ce que** les axes des rainures 3 dans la plaque supérieure 1 coïncident avec les axes des solides géométriques 4 qui y sont installés.

3. Blindage de protection passif en composite selon la revendication 1, **caractérisé en ce que** les solides géométriques 4 sont en céramique ou en métal.

4. Blindage de protection passif en composite selon la revendication 1, **caractérisé en ce que** les solides géométriques 4 ont la forme de sphères ou de pyramides tronquées à base carrée.
